



US008728695B2

(12) **United States Patent**  
**Kawakami et al.**

(10) **Patent No.:** **US 8,728,695 B2**  
(45) **Date of Patent:** **May 20, 2014**

(54) **ELECTROSTATIC CHARGE IMAGE DEVELOPING TONER, ELECTROSTATIC CHARGE IMAGE DEVELOPER, TONER CARTRIDGE, DEVELOPER CARTRIDGE, PROCESS CARTRIDGE, IMAGE FORMING APPARATUS, AND IMAGE FORMING METHOD**

(75) Inventors: **Eiji Kawakami**, Kanagawa (JP); **Shintaro Anno**, Kanagawa (JP); **Hirokazu Hamano**, Kanagawa (JP)

(73) Assignee: **Fuji Xerox Co., Ltd.**, Tokyo (JP)

(\*) Notice: Subject to any disclaimer, the term of this patent is extended or adjusted under 35 U.S.C. 154(b) by 0 days.

(21) Appl. No.: **13/560,599**

(22) Filed: **Jul. 27, 2012**

(65) **Prior Publication Data**

US 2013/0252161 A1 Sep. 26, 2013

(30) **Foreign Application Priority Data**

Mar. 23, 2012 (JP) ..... 2012-067657

(51) **Int. Cl.**  
**G03G 9/097** (2006.01)

(52) **U.S. Cl.**  
USPC ..... **430/108.7**; 430/123.51; 430/108.6;  
399/159

(58) **Field of Classification Search**  
CPC ..... G03G 9/09708; G03G 9/09725; G03G  
9/09716

See application file for complete search history.

(56) **References Cited**

U.S. PATENT DOCUMENTS

6,057,073 A 5/2000 Hagiwara  
2004/0062568 A1 \* 4/2004 Nukada et al. ..... 399/159  
2010/0075242 A1 \* 3/2010 Kunii et al. ..... 430/108.6

FOREIGN PATENT DOCUMENTS

JP A-9-166885 6/1997

\* cited by examiner

*Primary Examiner* — Peter Vajda

(74) *Attorney, Agent, or Firm* — Oliff PLC

(57) **ABSTRACT**

An electrostatic charge image developing toner includes toner particles containing a colorant, a binder resin, and a release agent; and an external additive, wherein the external additive contains inorganic particles which include a compound represented by Formula (1) below on the surfaces thereof:



wherein in Formula (1), R<sup>1</sup> and R<sup>8</sup> each independently represents an alkyl group, R<sup>2</sup> to R<sup>7</sup> each independently represents an alkyl group or a substituted or unsubstituted phenyl group, and at least three groups of R<sup>2</sup> to R<sup>7</sup> each independently represents a substituted or unsubstituted phenyl group.

**19 Claims, No Drawings**

1

**ELECTROSTATIC CHARGE IMAGE DEVELOPING TONER, ELECTROSTATIC CHARGE IMAGE DEVELOPER, TONER CARTRIDGE, DEVELOPER CARTRIDGE, PROCESS CARTRIDGE, IMAGE FORMING APPARATUS, AND IMAGE FORMING METHOD**

**CROSS-REFERENCE TO RELATED APPLICATIONS**

This application is based on and claims priority under 35 USC 119 from Japanese Patent Application No. 2012-067657 filed Mar. 23, 2012.

**BACKGROUND**

**1. Technical Field**

The present invention relates to an electrostatic charge image developing toner, an electrostatic charge image developer, a toner cartridge, a developer cartridge, a process cartridge, an image forming apparatus, and an image forming method.

**2. Related Art**

A method such as electrophotography in which image information is visualized through an electrostatic charge image, is currently being used in various fields. In electrophotography, an electrostatic charge image (electrostatic latent image) is formed on the surface of a photoreceptor (image holding member) through charging and exposure processes; and the electrostatic latent image is developed using a developer containing a toner and visualized through transfer and fixing processes. As the developer used in this case, there is used a two-component developer including a toner and a carrier; and a single-component developer in which a magnetic toner or a nonmagnetic toner is used alone. In addition, as a preparation method of this toner, a kneading and pulverizing method is normally used in which a thermoplastic resin is melted and kneaded along with a pigment, a charge-controlling agent, and a release agent such as wax, cooled, finely pulverized, and classified. Optionally, during toner preparation, inorganic or organic particles for improving fluidity and a cleaning property may be added to the surface of toner particles.

**SUMMARY**

According to an aspect of the invention, there is provided an electrostatic charge image developing toner including: toner particles containing at least a colorant, a binder resin, and a release agent; and an external additive, wherein the external additive contains inorganic particles which include a compound represented by Formula (1) below on the surfaces thereof:



wherein in Formula (1),  $\text{R}^1$  and  $\text{R}^8$  each independently represents an alkyl group,  $\text{R}^2$  to  $\text{R}^7$  each independently represents an alkyl group or a substituted or unsubstituted phenyl group,

2

and at least three groups of  $\text{R}^2$  to  $\text{R}^7$  each independently represents a substituted or unsubstituted phenyl group.

**DETAILED DESCRIPTION**

5

Hereinafter, an exemplary embodiment of the invention will be described.

**Electrostatic Charge Image Developing Toner**

An electrostatic charge image developing toner according to the exemplary embodiment (hereinafter, sometimes simply referred to as "the toner") includes toner particles containing a colorant, a binder resin, and a release agent; and an external additive, in which the external additive contains inorganic particles which include a compound represented by Formula (1) below on the surfaces thereof.



25 In Formula (1),  $\text{R}^1$  and  $\text{R}^8$  each independently represents an alkyl group, zero to three of  $\text{R}^2$  to  $\text{R}^7$  each independently represents an alkyl group, and three to six of  $\text{R}^2$  to  $\text{R}^7$  each independently represents a phenyl group.

The present inventors have found that, in toners of the 30 related art such as a toner disclosed in JP-A-9-166885, the surfaces of color particles or the surface of a carrier is coated with silicone oil used as an external additive, through mechanical stress caused by agitation in a developer unit or the like; due to moisture absorbency of the silicone oil in a high-temperature and high-humidity environment, moisture is attached to the surfaces of the color particles or the surface of the carrier and thus electric charge leaks from a moisture-attached site; and as a result, the charge amount deteriorates 35 after being left to stand idle for a long period of time and image defects such as fogging are caused.

40 As a result of in-depth examination, the present inventors have found that when the toner includes inorganic particles, which include the compound represented by Formula (1) on the surfaces thereof, as an external additive, toner filming is suppressed and charging stability is excellent even in a high-temperature and high-humidity environment.

45 It is presumed that the aromatic rings of the siloxane compound represented by Formula (1) are attracted to each other (presumably, by  $\pi$ - $\pi$  stacking forces); therefore, deposited materials are stably and uniformly formed on a contact portion (blade nip portion) between a cleaning blade and a photoreceptor; and as a result, a stable cleaning property may be obtained and toner filming is suppressed.

50 In addition, it is presumed that, when coating is performed using the siloxane compound represented by Formula (1), an oxygen atom in a main chain forms a hydrogen bond with a hydrogen atom in moisture attached to the surface of a toner or a carrier and thus a bulky aromatic ring is oriented toward the outside; therefore, water molecule adsorption is hindered 55 due to a steric barrier and formation of electric charge leakage sites is prevented; and as a result, charging stability is excellent and image defects such as fogging are suppressed.

**External Additive**

60 The electrostatic charge image developing toner according to the exemplary embodiment contains toner particles and an external additive. The external additive contains the inorganic

particles which include the compound represented by Formula (1) on the surfaces thereof.

With regard to the inorganic particles which include the compound represented by Formula (1) on the surfaces thereof, at least a part of the surfaces of the inorganic particles may be coated with the compound represented by Formula (1). However, it is preferable that 50% by area or more of the surfaces of the inorganic particles are coated with the compound represented by Formula (1) and it is more preferable that 80% by area or more of the surfaces of the inorganic particles are coated with the compound represented by Formula (1). As a method of measuring the coating amount of the compound represented by Formula (1), for example, a method is used in which the compound represented by Formula (1) is dyed with a colorant formed of an organic compound or an aromatic compound and the average value of 50 or more inorganic particles is calculated by imaging the toner or the inorganic particles and analyzing the image.

In addition, the compound represented by Formula (1) is attached to the surfaces of the inorganic particles. That is, the compound represented by Formula (1) may be physically adsorbed or bonded by a chemical bond to the surfaces of the inorganic particles. However, it is preferable that the compound represented by Formula (1) be physically adsorbed to the surfaces of the inorganic particles. According to the above-described example, even when the toner is exposed to a high-temperature and high-humidity environment for a long time, toner filming is more suppressed. In addition, when the compound represented by Formula (1) is physically adsorbed, the compound represented by Formula (1) is partially liberated or directly attached from the inorganic particles to a carrier, a photoreceptor, or the like, thereby further suppressing toner filming and more excellent charging stability is obtained.

#### Compound Represented by Formula (1)

The electrostatic charge image developing toner according to the exemplary embodiment contains the inorganic particles, which includes the compound represented by Formula (1) below on the surfaces thereof, as an external additive. When the toner contains the inorganic particles, which includes the compound represented by Formula (1) below (in which a phenyl group is included and only three silicon atoms are bonded through an oxygen atom) on the surfaces thereof, as an external additive, an electrostatic charge image developing toner is obtained in which toner filming is suppressed and charging stability is excellent even in a high-temperature and high-humidity environment.



In Formula (1),  $\text{R}^1$  and  $\text{R}^8$  each independently represents an alkyl group,  $\text{R}^2$  to  $\text{R}^7$  each independently represents an alkyl group or a substituted or unsubstituted phenyl group, and three to six of  $\text{R}^2$  to  $\text{R}^7$  each independently represents a substituted or unsubstituted phenyl group.

In Formula (1), as the alkyl group which is independently represented by  $\text{R}^1$  and  $\text{R}^8$  each, an alkyl group having from 1 to 20 carbon atoms is preferable, an alkyl group having from 1 to 8 carbon atoms is more preferable, an alkyl group having from 1 to 4 carbon atoms is still more preferable, and a methyl group is even still more preferable. According to the above-

described aspect, even in a high-temperature and high-humidity environment, toner filming is more suppressed and charging stability is superior.

In Formula (1), among  $\text{R}^2$  to  $\text{R}^7$ , it is preferable that one to three thereof each independently represents an alkyl group, it is more preferable that one or two thereof each independently represents an alkyl group, and it is still more preferable that one thereof represents an alkyl group. According to the above-described aspect, even in a high-temperature and high-humidity environment, charging stability is more excellent.

As the alkyl group represented by  $\text{R}^2$  to  $\text{R}^7$  in Formula (1), an alkyl group having from 1 to 20 carbon atoms is preferable, an alkyl group having from 1 to 8 carbon atoms is more preferable, an alkyl group having from 1 to 4 carbon atoms is still more preferable, and a methyl group is even still more preferable. According to the above-described aspect, even in a high-temperature and high-humidity environment, toner filming is suppressed and charging stability is more excellent.

The alkyl group represented by  $\text{R}^1$  to  $\text{R}^8$  may have a linear, branched, or cyclic structure.

Among  $\text{R}^2$  to  $\text{R}^7$  in Formula (1), it is preferable that three to five thereof each independently represents a substituted or unsubstituted phenyl group, it is more preferable that four or five thereof each independently represents a substituted or unsubstituted phenyl group, and it is still more preferable that five thereof each represents a substituted or unsubstituted phenyl group. According to the above-described aspect, even in a high-temperature and high-humidity environment, charging stability is more excellent.

The phenyl group represented by  $\text{R}^2$  to  $\text{R}^7$  may have a substituent, but it is preferable that the phenyl group does not have a substituent. Examples of the substituent include an alkyl group, an aryl group, an alkoxy group, an acyloxy group, an acyl group, and an alkyloxycarbonyl group.

In addition, among  $\text{R}^2$  to  $\text{R}^7$  in Formula (1), it is preferable that at least  $\text{R}^5$  represents an alkyl group, it is more preferable that  $\text{R}^4$  and  $\text{R}^5$ , or  $\text{R}^5$  represents an alkyl group, and it is still more preferable that only  $\text{R}^5$  represents an alkyl group. According to the above-described aspect, even in a high-temperature and high-humidity environment, charging stability is more excellent.

In addition, among  $\text{R}^2$  to  $\text{R}^7$  in Formula (1), it is preferable that  $\text{R}^3$  and  $\text{R}^7$  each independently represents a phenyl group.

Specifically, preferable examples of the compound represented by Formula (1) include 1,1,3,5,5-pentaphenyl-1,3,5-trialkyl trisiloxane, 1,1,5,5-tetraphenyl-1,3,3,5-tetraalkyl trisiloxane, 1,1,3,3,5,5-hexaphenyl-1,5-dialkyl trisiloxane, 1,1,3,3,5-pentaphenyl-1,5,5-trialkyl trisiloxane, 1,1,3,5-tetraphenyl-1,3,5,5-tetraalkyl trisiloxane, 1,3,3,5-tetraphenyl-1,5,5-tetraalkyl trisiloxane, 1,3,5-triphenyl-1,1,3,5,5-pentaalkyl trisiloxane, and 1,1,5-triphenyl-1,3,3,5,5-pentaalkyl trisiloxane, more preferable examples thereof include 1,1,3,5,5-pentaphenyl-1,3,5-trialkyl trisiloxane and 1,1,5,5-tetraphenyl-1,3,3,5-tetraalkyl trisiloxane, still more preferable examples thereof include 1,1,3,5,5-pentaphenyl-1,3,5-trimethyl trisiloxane and 1,1,5,5-tetraphenyl-1,3,3,5-tetramethyl trisiloxane, and an even still more preferable example includes 1,1,3,5,5-pentaphenyl-1,3,5-trimethyl trisiloxane. Inorganic Particles

The inorganic particles which include the compound represented by Formula (1) on the surfaces thereof are not particularly limited and inorganic particles well known as an external additive of the toner are used, and examples thereof include particles of silica, alumina, titanium oxides (for example, titanium oxide and metatitanic acid), cerium oxide, zirconia, calcium carbonate, magnesium carbonate, calcium phosphate, and carbon black.

Among these, silica particles or titanium oxide particles are preferable and silica particles are particularly preferable.

Examples of silica particles include particles of fumed silica, colloidal silica, and silica gel.

In addition to the fact that the inorganic particles include the compound represented by Formula (1) on the surfaces thereof, the surfaces of the inorganic particles may be treated with a silane coupling agent described below and the like, for example.

The volume average primary particle size of the inorganic particles is preferably from 3 nm to 500 nm, more preferably from 7 nm to 300 nm, still more preferably from 20 nm to 200 nm, and even still more preferably from 40 nm to 130 nm. In the above-described range, a transfer property of the compound represented by Formula (1) to a carrier, a photoreceptor, and the like is excellent and toner filming is further suppressed.

It is preferable that the volume average primary particle size of the inorganic particles be measured using an LS13-320 (manufactured by Beckman Coulter Inc.).

In addition, in the toner according to the exemplary embodiment, it is preferable that the volume average primary particle size of the inorganic particles, which include the compound represented by Formula (1) on the surfaces thereof, be greater than that of other external additives except the inorganic particles.

In the toner according to the exemplary embodiment, the content of the inorganic particles which include the compound represented by Formula (1) on the surfaces thereof is not particularly limited, but preferably from 0.3% by weight to 10% by weight, more preferably from 0.5% by weight to 4% by weight, and still more preferably from 0.8% by weight to 2.0% by weight, with respect to the total weight of the toner. Preparation Method of Inorganic Particles Including Compound Represented by Formula (1) On Surfaces Thereof (Surface Treatment Method)

The preparation method of the inorganic particles including the compound represented by Formula (1) on the surfaces thereof is not particularly limited and well-known methods are used. In addition, a chemical process is not necessarily performed. Even when the compound represented by Formula (1) is physically adsorbed to the surfaces of the inorganic particles, an effect of the exemplary embodiment is exhibited sufficiently.

Examples of the physical adsorption method include a dry method such as a spray dry method in which the compound represented by Formula (1) or a liquid containing the compound represented by Formula (1) is sprayed on inorganic particles floating in the gas phase and a method in which inorganic particles are dipped in a solution containing the compound represented by Formula (1) and dried. In addition, the compound represented by Formula (1) on the surfaces of the inorganic particles may be chemically treated by heating the inorganic particles subjected to the physical adsorption.

In the toner according to the exemplary embodiment, the amount of the compound represented by Formula (1) with which inorganic particles are treated (the content of the compound represented by Formula (1) in the toner) is preferably equal to or greater than 0.16% by weight and more preferably equal to or greater than 0.26% by weight; and preferably less than or equal to 5% by weight, more preferably less than or equal to 1% by weight, and still more preferably less than or equal to 0.50% by weight, with respect to the total weight of the toner. In the above-described range, an effect of suppressing toner filming is more greatly exhibited.

As a method of externally adding the external additive to the toner according to the exemplar embodiment, for

example, a method is used in which toner particles and external additives are mixed using a Henschel mixer or a V-blender. In addition, when the toner particles are prepared in a wet method, the external additive may be externally added in a wet method.

In addition, for example, a method is used in which the inorganic particles are added to the toner particles, the compound represented by Formula (1) or a liquid containing the compound represented by Formula (1) is added thereto, and the resultant is mixed using a Henschel mixer or a V-blender.

Among these methods, the physical adsorption method is preferable as the preparation method of the inorganic particles including the compound represented by Formula (1) on the surfaces thereof.

#### Other External Additives

The toner according to the exemplary embodiment may contain other external additives except the inorganic particles including the compound represented by Formula (1) on the surfaces thereof (hereinafter, also referred to as "other external additives").

The content of other external additives in the toner according to the exemplary embodiment may be less than that of the inorganic particles including the compound represented by Formula (1) on the surfaces thereof.

Examples of other external additives include the above-described inorganic particles, resin particles of vinyl resin, polyester resin, and silicone resin.

It is preferable that the surfaces of the inorganic particles used as other external additives be treated with a hydrophobizing agent in advance. This hydrophobizing treatment is effective for improving powder fluidity of a toner, dependency of electric charging on an environment, and contamination resistance of a carrier.

The hydrophobizing treatment may be performed by, for example, dipping the inorganic particles in a hydrophobizing agent. The hydrophobizing agent is not particularly limited and examples thereof include a silane coupling agent, a titanate coupling agent, and an aluminum coupling agent. These hydrophobizing agents may be used alone or in a combination of two or more kinds thereof. Among these, the silane coupling agent is preferable.

As the silane coupling agent, for example, any type of chlorosilane, alkoxy silane, silazane, and a special silylating agent may be used.

Specific examples thereof include methyltrichlorosilane, dimethyldichlorosilane, trimethylchlorosilane, phenyltrichlorosilane, diphenyldichlorosilane, tetramethoxysilane, methyltrimethoxysilane, dimethyldimethoxysilane, phenyltrimethoxysilane, diphenyldimethoxysilane, tetraethoxysilane, methyltrioethoxysilane, dimethyldioethoxysilane, phenyltrioethoxysilane, diphenyldioethoxysilane, isobutyltrioethoxysilane, decyltrimethoxysilane, hexamethyldisilazane, N,O-(bistrimethylsilyl)acetamide, N,N-(trimethylsilyl)urea, tert-butyldimethylchlorosilane, vinyltrichlorosilane, vinyltrimethoxysilane, vinyltriethoxysilane,  $\gamma$ -methacryloxypropyltrimethoxysilane,  $\beta$ -(3,4-epoxycyclohexyl)ethyltrimethoxysilane,  $\gamma$ -glycidoxypropyltrimethoxysilane,  $\gamma$ -glycidoxypropylmethyldioethoxysilane,  $\gamma$ -mercaptopropyltrimethoxysilane, and  $\gamma$ -chloropropyltrimethoxysilane.

The content of the hydrophobizing agent varies depending on the kind of the inorganic particles and is difficult to define indiscriminately, but is preferably from 1 part by weight to 50 parts by weight and more preferably from 5 parts by weight to 20 parts by weight, with respect to 100 parts by weight of the

inorganic particles. In the exemplary embodiment, as the hydrophobic silica particles, commercially available products are preferably used.

The average primary particle size of other external additives is preferably from 3 nm to 500 nm, more preferably from 5 nm to 100 nm, still more preferably from 5 nm to 50 nm, and even still more preferably from 5 nm to 40 nm.

#### Toner Particles

The electrostatic charge image developing toner according to the exemplary embodiment includes toner particles containing a colorant, a binder resin, and a release agent. In addition, the toner particles further include well-known external additives such as a charge-controlling agent.

#### Binder Resin

Examples of the binder resin include polyolefin resin such as polyethylene or polypropylene, styrene resin including polystyrene and poly( $\alpha$ -methylstyrene) as a major component, (meth)acrylic resin including polymethyl methacrylate and polyacrylonitrile as a major component, styrene-(meth)acrylic copolymer resin, polyamide resin, polycarbonate resin, polyether resin, polyester resin, and a copolymer resin thereof. However, from the viewpoints of charging stability and development durability when used for the electrostatic charge image developing toner, styrene resin, (meth)acrylic resin, styrene-(meth)acrylic copolymer resin, and polyester resin are preferable.

As the binder resin, from the viewpoint of a low-temperature fixing property, a binder resin containing polyester resin is preferable and a binder resin containing amorphous (non-crystalline) polyester resin is more preferable.

Polyester resin is a resin obtained by polycondensation of polyvalent carboxylic acids and polyols mainly.

Examples of polyvalent carboxylic acids include aromatic carboxylic acids such as terephthalic acid, isophthalic acid, phthalic anhydride, trimellitic anhydride, pyromellitic acid, and naphthalenedicarboxylic acid; aliphatic carboxylic acids such as maleic anhydride, fumaric acid, succinic acid, alkenyl succinic anhydride, and adipic acid; alicyclic carboxylic acids such as cyclohexanedicarboxylic acid; and lower alkyl esters and acid anhydrides thereof. Lower alkyl represents a linear, branched, or cyclic alkyl group having from 1 to 8 carbon atoms. These polyvalent carboxylic acids are used alone or in a combination of two or more kinds thereof. Among these polyvalent carboxylic acids, aromatic carboxylic acids are preferably used. In addition, in order to adopt a cross-linked structure or a branched structure for obtaining an excellent fixing property, it is preferable that a dicarboxylic acid be used in combination with a trivalent or higher carboxylic acid (for example, trimellitic acid and acid anhydride thereof).

Examples of polyvalent carboxylic acids used for obtaining amorphous polyester resin include aromatic dicarboxylic acids such as phthalic acid, isophthalic acid, terephthalic acid, naphthalene-2,6-dicarboxylic acid, 1,4-phenylenediacetic acid, and 1,4-cyclohexanedicarboxylic acid; dicarboxylic acids having an alicyclic hydrocarbon group; and acid anhydrides and lower alkyl esters thereof.

Examples of polyols include aliphatic diols such as ethylene glycol, diethylene glycol, triethylene glycol, propylene glycol, butanediol, hexanediol, neopentyl glycol, and glycerin; alicyclic diols such as cyclohexanediol, cyclohexanediethanol, and hydrogenated bisphenol A; and aromatic diols such as ethylene oxide adducts of bisphenol A and propylene oxide adducts of bisphenol A. These polyols may be used alone or in a combination of two or more kinds thereof.

As polyols used for obtaining amorphous polyester, for example, aliphatic, alicyclic, and aromatic polyols are preferable, and specific examples thereof include 1,4-cyclohexanediol, 1,4-cyclohexanediethanol, alkylene oxide adducts of bisphenol A, alkylene oxide adducts of bisphenol Z, and alkylene oxide adducts of hydrogenated bisphenol A. Among these, alkylene oxide adducts of bisphenol A are preferably used, and ethylene oxide 2 mol adduct of bisphenol A and propylene oxide 2 mol adduct of bisphenol A are more preferably used.

In addition, in order to adopt a cross-linked structure or a branched structure for obtaining a further excellent fixing property, it is preferable that diols be used in combination with trivalent or higher alcohols (for example, glycerin, trimethylolpropane, and pentaerythritol).

The glass transition temperature (hereinafter, may be abbreviated as "Tg") of amorphous polyester resin is preferably from 50°C. to 80°C. and more preferably from 50°C. to 70°C. When Tg is lower than or equal to 80°C., a low-temperature fixing property is excellent, which is preferable. In addition, when Tg is equal to or higher than 50°C., heat-resistant preservability is excellent and the preservability of a fixed image is also excellent, which is preferable.

The acid value of amorphous polyester resin is preferably from 5 mg KOH/g to 25 mg KOH/g and more preferably from 6 mg KOH/g to 23 mg KOH/g. When the acid value is equal to or greater than 5 mg KOH/g, the affinity of toner for paper and a charging property are excellent. In addition, when the toner is prepared using an emulsion aggregation method described below, emulsified particles are easily prepared, the aggregation speed of an aggregation process and the rate of change of shape in a coalescence process in the emulsion aggregation method are suppressed from significantly increasing, thereby making a particle size control and shape control easy. In addition, when the acid value of amorphous polyester resin is less than or equal to 25 mg KOH/g, there is no adverse effect on dependency of electric charging on an environment. In addition, when toner is prepared in the emulsion aggregation method, the aggregation speed of the aggregation process and the speed of change of shape in the coalescence process are suppressed from significantly decreasing, thereby preventing deterioration in productivity.

When the molecular weight of a tetrahydrofuran (THF)-soluble matter of amorphous polyester resin is measured using a gel permeation chromatography (GPC) method, the weight average molecular weight (Mw) is preferably from 5,000 to 1,000,000 and more preferably from 7,000 to 500,000; the number average molecular weight (Mn) is from 2,000 to 100,000; and the molecular weight distribution Mw/Mn is preferably from 1.5 to 100 and more preferably from 2 to 60.

When the molecular weight and the molecular weight distribution of amorphous polyester resin is in the above-described range, a low-temperature fixing property does not deteriorate and the fix level of an image is excellent, which is preferable.

In the exemplary embodiment, the toner particles may contain crystalline polyester resin.

Crystalline polyester resin is compatible with amorphous polyester resin when dissolved and thereby toner viscosity deteriorates significantly. As a result, a toner having a further excellent low-temperature fixing property may be obtained. Among crystalline polyester resins, most crystalline aromatic polyester resins have the melting points that are generally higher than a melting temperature range described below. Therefore, when crystalline polyester resin is included, crystalline aliphatic polyester resin is preferable.

In the exemplary embodiment, the content of crystalline polyester resin in the toner particles is preferably from 2% by weight to 30% by weight and more preferably from 4% by weight to 25% by weight. When the content is equal to or greater than 2% by weight, the viscosity of amorphous polyester resin may be reduced when dissolved, thereby easily improving a low-temperature fixing property. When the content is less than or equal to 30% by weight, deterioration of the charging property of toner, which is caused by the presence of crystalline polyester resin, is prevented and furthermore, after an image is fixed onto a recording medium, a high fix level of the image is easily obtained.

The melting temperature of crystalline polyester resin is preferably from 50°C. to 90°C., more preferably from 55°C. to 90°C., and still more preferably from 60°C. to 90°C. When the melting temperature is equal to or higher than 50°C., toner preservability and the preservability of a fixed toner image are excellent. When the melting temperature is lower than or equal to 90°C., a low-temperature fixing property is improved.

The glass transition temperature (Tg) of amorphous polyester resin is preferably equal to or higher than 30°C., more preferably from 30°C. to 100°C., and still more preferably from 50°C. to 80°C. In the above-described range, since amorphous polyester resin is used in a glass state, the toner particles are not aggregated by heat or pressure applied during image formation and are not attached and deposited in an image forming apparatus. As a result, a stable image forming function may be obtained over a long period of time.

The glass transition temperature of resin may be measured using well-known methods, for example, a method defined by ASTM D3418-82 (DSC method).

The melting temperature of crystalline resin is measured using a differential scanning calorimeter (DSC) and can be obtained as a melting peak temperature when the measurement is performed using input compensation differential scanning calorimetry shown in JIS K-7121 while the temperature is raised from room temperature to 150°C. at a rate of temperature increase of 10°C./min.

"The crystallinity" of crystalline resin represents that a clear endothermic peak, not a stepwise endothermic change, is shown in the differential scanning calorimetry (DSC) and specifically represents that the half width of an endothermic peak when measured at a rate of temperature increase of 10°C./min is within 15°C.

On the other hand, a resin in which the half width of an endothermic peak is higher than 15°C. and a resin in which a clear endothermic peak is not shown are defined as noncrystalline (amorphous) resin. The glass transition temperature of amorphous resin is measured using a differential scanning calorimeter (DSC-50, manufactured by Shimadzu Corporation) which is equipped with an automatic tangent line processing system according to ASTM D3418. Measurement conditions are as follows.

Sample: 3 mg to 15 mg, preferably 5 mg to 10 mg

Measurement method: a sample is put into an aluminum pan and an empty aluminum pan is prepared for reference.

Temperature curve: Temperature Rise I (20°C. to 180°C., a rate of temperature increase of 10°C./min)

The glass transition temperature is measured from an endothermic curve which is measured during a temperature rise in the temperature curve.

The glass transition temperature is a temperature in which a differential value of the endothermic curve is maximum.

In addition, when crystalline polyester resin is a polymer in which other components are copolymerized with a main

chain thereof and there are less than 50% by weight of other components, this copolymer is also called crystalline polyester.

As acid components used for synthesizing crystalline polyester resin, for example, various polyvalent carboxylic acids are used, but dicarboxylic acids are preferable and linear aliphatic dicarboxylic acids are more preferable.

Examples thereof include oxalic acid, malonic acid, succinic acid, glutaric acid, adipic acid, pimelic acid, suberic acid, azelaic acid, sebatic acid, 1,9-nonanedicarboxylic acid, 1,10-decanedicarboxylic acid, 1,11-undecanedicarboxylic acid, 1,12-dodecanedicarboxylic acid, 1,13-tridecanedicarboxylic acid, 1,14-tetradecanedicarboxylic acid, 1,16-hexadecanedicarboxylic acid, 1,18-octadecanedicarboxylic acid, and lower alkyl esters and acid anhydrides thereof. However, the acid components are not limited to these examples. Among these, adipic acid, sebatic acid, and 1,10-decanedicarboxylic acid are preferable in consideration of availability.

In addition, as the acid components used for synthesizing crystalline polyester resin, dicarboxylic acids having an ethylenic unsaturated bond and dicarboxylic acids having a sulfonic acid group may be used.

As alcohol components used for synthesizing crystalline polyester resin, aliphatic diols are preferable, and examples thereof include ethylene glycol, 1,3-propanediol, 1,4-butanediol, 1,5-pentanediol, 1,6-hexanediol, 1,7-heptanediol, 1,8-octanediol, 1,9-nonanediol, 1,10-decanediol, 1,11-dodecanediol, 1,12-undecanediol, 1,13-tridecanediol, 1,14-tetradecadiol, 1,18-octadecanediol, and 1,20-eicosanediol. However, the alcohol components are not limited to these examples. Among these, 1,4-butanediol, 1,6-hexanediol, 1,8-octanediol, 1,9-nonanediol, and 1,10-decanediol are preferable in consideration of availability and cost.

The molecular weight (weight average molecular weight, Mw) of crystalline polyester resin is preferably from 8,000 to 40,000 and more preferably from 10,000 to 30,000, from the viewpoints of manufacturability of the resin, fine dispersion during toner preparation, and compatibility during dissolving. When the weight average molecular weight is equal to or greater than 8,000, the reduction in the electric resistance of crystalline polyester resin is suppressed, thereby preventing deterioration in charging property. In addition, when the weight average molecular weight is less than or equal to 40,000, a cost for synthesizing the resin is suppressed and deterioration of a sharp melting property is prevented. As a result, there is no adverse effect on a low-temperature fixing property.

In the exemplary embodiment, the molecular weight of polyester resin is measured using GPC (Gel Permeation Chromatography) and calculated. Specifically, an HLC-8120 (manufactured by TOSOH CORPORATION) is used for the GPC, a TSK gel Super HM-M (15 cm, manufactured by TOSOH CORPORATION) is used as a column, and polyester resin is measured in a THF solvent. Next, the molecular weight of polyester resin is calculated using a molecular weight calibration curve prepared from monodisperse polystyrene standard samples.

The preparation method of polyester resin is not particularly limited and a general polyester polymerization method in which acid components and alcohol components are caused to react with each other may be used. For example, a direct polycondensation method, an ester exchange method, and the like are used depending on the kinds of monomers.

The mole ratio (acid components/alcohol components) when the acid components and the alcohol components are caused to react with each other varies depending on reaction condi-

## 11

tions and the like and thus is difficult to define indiscriminately, but is preferably about 1/1 in general in order to obtain a high molecular weight.

Examples of a catalyst which may be used during polyester resin preparation include a compound of an alkali metal such as sodium or lithium; a compound of an alkaline earth metal such as magnesium or calcium; a compound of metals such as zinc, manganese, antimony, titanium, tin, zirconium, or germanium; a phosphite compound; a phosphate compound; and an amine compound.

Styrene resin and (meth)acrylic resin, and in particular, styrene-(meth)acrylic copolymer resin are useful as the binder resin in the exemplary embodiment.

A monomer mixture, which is obtained by mixing 60 parts by weight to 90 parts by weight of vinyl aromatic monomer (styrene monomer), 10 parts by weight to 40 parts by weight of ethylenically unsaturated carboxylic acid ester monomer ((meth)acrylic ester monomer), and 1 part by weight to 3 parts by weight of ethylenically unsaturated acid monomer, is polymerized to obtain a copolymer, and a latex in which the obtained copolymer is dispersed and stabilized by a surfactant is preferably used as a binder resin component.

The glass transition temperature of the above copolymer is preferably from 50° C. to 70° C.

Hereinafter, polymerizable monomers constituting the above copolymer resin will be described.

Examples of styrene monomer include styrene;  $\alpha$ -methylstyrene; vinylnaphthalene; alkyl-substituted styrene having an alkyl chain such as 2-methylstyrene, 3-methylstyrene, 4-methylstyrene, 2-ethylstyrene, 3-ethylstyrene, or 4-ethylstyrene; halogen-substituted styrene such as 2-chlorostyrene, 3-chlorostyrene, or 4-chlorostyrene; and fluorine-substituted styrene such as 4-fluorostyrene or 2,5-difluorostyrene. Among these, styrene is preferable as the styrene monomer.

Examples of (meth)acrylic acid ester monomer include n-methyl(meth)acrylate, n-ethyl(meth)acrylate, n-propyl (meth)acrylate, n-butyl(meth)acrylate, n-pentyl(meth)acrylate, n-hexyl(meth)acrylate, n-heptyl(meth)acrylate, n-octyl (meth)acrylate, n-decyl(meth)acrylate, n-dodecyl(meth)acrylate, n-lauryl(meth)acrylate, n-tetradecyl(meth)acrylate, n-hexadecyl(meth)acrylate, n-octadecyl(meth)acrylate, isopropyl(meth)acrylate, isobutyl(meth)acrylate, t-butyl(meth)acrylate, isopentyl(meth)acrylate, amyl(meth)acrylate, neopentyl(meth)acrylate, isohexyl(meth)acrylate, isoheptyl (meth)acrylate, isoctyl(meth)acrylate, 2-ethylhexyl(meth)acrylate, phenyl(meth)acrylate, biphenyl(meth)acrylate, diphenylethyl(meth)acrylate, t-butylphenyl(meth)acrylate, terphenyl(meth)acrylate, cyclohexyl(meth)acrylate, t-butylcyclohexyl(meth)acrylate, dimethylaminoethyl(meth)acrylate, diethylaminoethyl(meth)acrylate, methoxyethyl(meth)acrylate, 2-hydroxyethyl(meth)acrylate,  $\beta$ -carboxyethyl (meth)acrylate, (meth)acrylonitrile, and (meth)acrylamide. Among these, n-butyl acrylate is preferable as the (meth)acrylic acid ester monomer.

The ethylenically unsaturated acid monomer contains a carboxyl group, a sulfonate group, and an acid group such as acid anhydride.

When a carboxyl group is to be contained in styrene resin, (meth)acrylic resin or styrene-(meth)acrylic copolymer resin, the carboxyl group-containing resin may be obtained by copolymerization of a polymerizable monomer having a carboxyl group.

Specific examples of such a polymerizable monomer having a carboxyl group include acrylic acid, aconitic acid, atropic acid, allylmalonic acid, angelic acid, isocrotonic acid, itaconic acid, 10-undecenoic acid, elaidic acid, erucic acid, oleic acid, o-carboxylic acid, crotonic acid, chloro-

## 12

acrylic acid, chloroisocrotonic acid, chlorocrotonic acid, chlorofumaric acid, chloromaleic acid, cinnamic acid, cyclohexenedicarboxylic acid, citraconic acid, hydroxycinnamic acid, dihydroxycinnamic acid, tiglic acid, nitrocinnamic acid, vinylacetic acid, phenylcinnamic acid, 4-phenyl-3-butenoic acid, ferulic acid, fumaric acid, brassidic acid, 2-(2-furyl) acrylic acid, bromocinnamic acid, bromofumaric acid, bromomaleic acid, benzylidenemalonic acid, benzylacrylic acid, 4-pentenoic acid, maleic acid, measaconic acid, methacrylic acid, methylcinnamic acid, and methoxycinnamic acid. Among these, in view of the case of a polymerization reaction, acrylic acid, methacrylic acid, maleic acid, cinnamic acid, and fumaric acid are preferable, and acrylic acid is more preferable.

15 The binder resin may use a chain-transfer agent for polymerization thereof.

The chain-transfer agent is not particularly limited, and a compound having a thiol component may be used. Specifically, alkyl mercaptans such as hexyl mercaptan, heptyl mercaptan, octyl mercaptan, nonyl mercaptan, decyl mercaptan, 20 and dodecyl mercaptan are preferable from the viewpoints of a narrow molecular weight distribution and accordingly excellent toner preservability at high temperature.

Optionally, the binder resin may contain a cross-linking agent. As a representative example of the cross-linking agent, a polyfunctional monomer having two or more ethylenically unsaturated groups in the molecule is used.

Specific examples of such a cross-linking agent include aromatic polyvinyl compounds such as divinylbenzene, and 30 divinylnaphthalene; polyvinyl esters of aromatic polyvalent carboxylic acid such as divinyl phthalate, divinyl isophthalate, divinyl terephthalate, divinyl homophthalate, divinyl/trivinyl trimesate, divinyl naphthalenedicarboxylate, and divinyl biphenylcarboxylate; divinyl esters of a nitrogen-containing aromatic compound such as divinyl pyridinedicarboxylate; vinyl esters of an unsaturated heterocyclic compound carboxylic acid such as vinyl pyromucinate, vinyl furancarboxylate, vinyl pyrrol-2-carboxylate, and vinyl thiophenecarboxylate; (meth)acrylate esters of linear polyols such as butanediol methacrylate, hexanediol acrylate, octanediol methacrylate, decanediol acrylate, and dodecanediol methacrylate; (meth)acrylate esters of branched or substituted polyols such as neopentyl glycol dimethacrylate and 40 2-hydroxy-1,3-diacyloxypropane; polyethylene glycol di(meth)acrylate and polypropylene polyethylene glycol di(meth)acrylate; and polyvinyl esters of polyvalent carboxylic acid such as divinyl succinate, divinyl fumarate, vinyl/divinyl maleate, divinyl diglycolate, vinyl/divinyl itaconate, divinyl acetonedicarboxylate, divinyl glutarate, divinyl 3,3'-thiodipropionate, divinyl/trivinyl trans-aconitate, divinyl adipate, divinyl pimelate, divinyl suberate, divinyl azelate, divinyl sebacate, divinyl dodecanedioate, and divinyl brassylate.

50 In the exemplary embodiment, these cross-linking agents may be used alone or in a combination of two or more kinds thereof.

The content of the cross-linking agent is preferably from 0.05% by weight to 5% by weight and more preferably from 0.1% by weight to 1.0% by weight, with respect to the total weight of polymerizable monomer.

60 Among the binder resins, a resin which may be prepared by radical polymerization of polymerizable monomers may be polymerized using a radical polymerization initiator.

The radical polymerization initiator is not particularly limited. Specific examples thereof include peroxides such as 65 hydrogen peroxide, acetyl peroxide, cumyl peroxide, tert-butyl peroxide, propionyl peroxide, benzoyl peroxide, chlorobenzoyl peroxide, dichlorobenzoyl peroxide, bromomethyl

benzoyl peroxide, lauroyl peroxide, ammonium persulfate, sodium persulfate, potassium persulfate, diisopropyl peroxy-carbonate, tetratin hydroperoxide, 1-phenyl-2-methyl propyl-1-hydroperoxide, tert-butyl triphenyl peracetate hydroperoxide, tert-butyl performate, tert-butyl peracetate, tert-butyl perbenzoate, tert-butyl phenyl peracetate, tert-butyl methoxy peracetate, and tert-butyl N-(3-toluoyl)percarbamate; azo compounds such as 2,2'-azobispropane, 2,2'-dichloro-2,2'-azobispropane, 1,1'-azo(methyl ethyl)diacetate, 2,2'-azobis(2-amidinopropane)hydrochloride, 2,2'-azobis(2-amidinopropane)nitrate, 2,2'-azobisisobutane, 2,2'-azobisisobutylamide, 2,2'-azobisisobutyronitrile, methyl 2,2'-azobis-2-methyl propionate, 2,2'-dichloro-2,2'-azobisbutane, 2,2'-azobis-2-methyl butyronitrile, dimethyl 2,2'-azobisisobutyrate, 1,1'-azobis(sodium 1-methyl butyronitrile-3-sulfonate), 2-(4-methyl phenylazo)-2-methyl malonodinitrile, 4,4'-azobis-4-cyanovaleate, 3,5-dihydroxymethyl phenylazo-2-methyl malonodinitrile, 2-(4-bromophenylazo)-2-allyl malonodinitrile, 2,2'-azobis-2-methyl valeronitrile, dimethyl 4,4'-azobis-4-cyanovaleate, 2,2'-azobis-2,4-dimethyl valeronitrile, 1,1'-azobiscyclohexane nitrile, 2,2'-azobis-2-propyl butyronitrile, 1,1'-azobis-1-chlorophenyl ethane, 1,1'-azobis-1-cyclohexane carbonitrile, 1,1'-azobis-1-cycloheptane nitrile, 1,1'-azobis-1-phenyl ethane, 1,1'-azobiscumene, ethyl 4-nitrophenylazobenzyl cyanoacetate, phenylazodiphenyl methane, phenylazotriphenyl methane, 4-nitrophenylazotriphenyl methane, 1,1'-azobis-1,2-diphenyl ethane, poly(bisphenol A-4,4'-azobis-4-cyanopentanoate), and poly(tetraethylene glycol-2,2'-azobisisobutyrate); 1,4-bis(pentaethylene)-2-tetrazene and 1,4-dimethoxycarbonyl-1,4-diphenyl-2-tetrazene.

In addition, examples of crystalline vinyl resin include vinyl resins which are prepared from alkyl or alkenyl esters of (meth)acrylic acid having a long chain such as amyl(meth)acrylate, hexyl(meth)acrylate, heptyl(meth)acrylate, octyl (meth)acrylate, nonyl(meth)acrylate, decyl(meth)acrylate, undecyl(meth)acrylate, tridecyl(meth)acrylate, myristyl (meth)acrylate, cetyl(meth)acrylate, stearyl(meth)acrylate, oleyl(meth)acrylate, and behenyl(meth)acrylate. In this specification, "(meth)acryl" represents any one of "acryl" and "methacryl" or both of them.

In addition, the weight average molecular weight of an addition polymerization resin such as styrene resin and (meth)acrylic resin is preferably from 5,000 to 50,000 and more preferably from 7,000 to 35,000. When the weight average molecular weight is equal to or greater than 5,000, cohesive force as the binder resin is excellent and a hot-offset property does not deteriorate. In addition, when the weight average molecular weight is less than or equal to 50,000, an excellent hot-offset property and minimum fixing temperature may be obtained. In addition, a time and a temperature required for polycondensation is appropriate and preparation efficiency is excellent.

In this case, the weight average molecular weight of the binder resin may be measured using, for example, gel permeation chromatography (GPO).

The content of the binder resin in the toner according to the exemplary embodiment is not particularly limited, but is preferably from 10% by weight to 95% by weight, more preferably from 25% by weight to 90% by weight, and still more preferably from 45% by weight to 85% by weight, with respect to the total weight of the toner. In the above-described range, a fixing property, a charging property, and the like are excellent.

## Colorant

The toner particles contain a colorant.

Examples of the colorant used for the toner according to the exemplary embodiment include magnetic powder such as magnetite or ferrite; various pigments such as Carbon Black, Lamp Black, Chrome Yellow, Hansa Yellow, Benzidine Yellow, Threne Yellow, Quinoline Yellow, Permanent Orange GTR, Pyrazolone Orange, Vulkan Orange, Watchyoung Red, Permanent Red, Brilliant Carmine 3B, Brilliant Carmine 6B, Du Pont Oil Red, Pyrazolone Red, Lithol Red, Rhodamine B Lake, Lake Red C, Rose Bengal, Aniline Blue, Ultramarine Blue, Calco Oil Blue, Methylene Blue Chloride, Phthalocyanine Blue, Phthalocyanine Green, and Malachite Green Oxalate; and various dyes of acridine, xanthene, azo, benzoinone, azine, anthraquinone, thioindigo, dioxadine, thiazine, azomethine, indigo, phthalocyanine, aniline black, polymethine, triphenylmethane, diphenylmethane, and thiazole. These examples may be used alone or in a combination of two or more kinds.

Furthermore, for example, C.I. Pigment Red 48:1, C.I. Pigment Red 122, C.I. Pigment Red 57:1, C.I. Pigment Yellow 97, C.I. Pigment Yellow 17, C.I. Pigment Blue 15:1, and C.I. Pigment Blue 15:3 are also used.

The content of the colorant in the toner particles according to the exemplary embodiment is preferably from 1 part by weight to 30 parts by weight with respect to 100 parts by weight of the binder resin included in the toner particles. In addition, optionally, use of a surface-treated colorant or a pigment dispersant may be effective. By appropriately selecting the kind of the colorant, various color toners such as yellow toner, magenta toner, cyan toner, and black toner may be obtained.

## Release Agent

The toner particles contain a release agent.

The release agent used in the exemplary embodiment is not particularly limited. Well-known release agents are used and waxes below are preferable.

Examples thereof include paraffin wax and derivatives thereof, montan wax and derivatives thereof, microcrystalline wax and derivatives thereof, Fischer-Tropsch wax and derivatives thereof, and polyolefin wax and derivatives thereof. The derivatives include polymers with oxide or vinyl monomers; and graft-modified products. As other examples, alcohol, fatty acid, vegetable wax, animal wax, mineral wax, ester wax and acid amide are also used.

The wax used as the release agent has a melting temperature of preferably from 70°C. to 140°C. and a melt viscosity of preferably from 1 centipoise to 200 centipoise and more preferably 1 centipoise to 100 centipoise. When the melting point is equal to or higher than 70°C., the change temperature of wax is sufficiently high. Therefore, blocking resistance and developability when a temperature in a copying machine is high are excellent. When the melting point is lower than or equal to 140°C., the change temperature of wax is sufficiently low. Therefore, it is not necessary to perform fixing at high temperature and power-saving characteristics are excellent. In addition, when the melt viscosity is less than or equal to 200 centipoise, elution from toner is appropriate, fixing and releasing properties are excellent.

In the toner according to the exemplary embodiment, the release agent is selected from the viewpoints of a fixing property, a toner blocking property, toner strength, and the like. The addition amount of the release agent is not particularly limited but is preferably from 2 parts by weight to 20 parts by weight with respect to 100 parts by weight of the binder resin included in the toner particles.

## Other Additives

Optionally, the toner particles may further include various components such as an internal additive or a charge-controlling agent, in addition to the above-described components.

Examples of the internal additive include metals such as ferrite, magnetite, reduced iron, cobalt, nickel, or manganese, alloys thereof, and magnetic materials such as compounds including the above-described metals.

Examples of the charge-controlling agent include a quaternary ammonium salt compound, a nigrosine-based compound, a dye formed of a complex of aluminum, iron and chromium, and triphenylmethane pigment.

The preparation method of the toner particles used in the exemplary embodiment is not particularly limited and well-known methods may be used. Specific examples of the preparation method of the toner particles are as follows: a kneading and pulverizing method in which the binder resin, the colorant, and the release agent (optionally, the charge-controlling agent and the like) are kneaded, pulverized, and classified; a method in which shapes of particles obtained using the kneading and pulverizing method are changed by mechanical shock or heat energy; an emulsion aggregation method in which a dispersion having the binder resin emulsified and dispersed therein and a dispersion having the colorant and the release agent (optionally, the charge-controlling agent and the like) are mixed, aggregated, heated, and coalesced to obtain toner particles; an emulsion polymerization aggregation method in which a dispersion obtained by emulsifying and polymerizing a polymerizable monomer of the binder resin, and a dispersion having the colorant, and the release agent (optionally, the charge-controlling agent and the like) are mixed, aggregated, heated, and coalesced to obtain toner particles; a suspension polymerization method in which a polymerizable monomer for obtaining the binder resin and a solution having the colorant, and the release agent (optionally, the charge-controlling agent and the like) are suspended in an aqueous solvent and polymerized; and a dissolving suspension method in which the binder resin and a solution having the colorant, and the release agent (optionally, the charge-controlling agent and the like) are suspended in an aqueous solvent and polymerized for granulation. In addition, a preparation method may be used in which the toner particles obtained in the above method are used as a core and furthermore aggregated particles are attached, heated, and coalesced to have a core-shell structure.

Among these, it is preferable that the toner according to the exemplary embodiment be toner (emulsion aggregation toner) obtained in the emulsion aggregation method or an emulsion polymerization aggregation method.

The volume average particle size of the toner particles obtained as described above is preferably from 2  $\mu\text{m}$  to 8  $\mu\text{m}$  and more preferably from 3  $\mu\text{m}$  to 7  $\mu\text{m}$ . When the volume average particle size is equal to or greater than 2  $\mu\text{m}$ , the liquidity of the toner is excellent and sufficient charging capability is imparted from a carrier, thereby suppressing background fogging and deterioration of density reproduction. In addition, when the volume average particle size is less than or equal to 8  $\mu\text{m}$ , fine dot reproduction, tone, and graininess are significantly improved, thereby obtaining a high-quality image. The volume average particle size is measured using a measuring machine such as Coulter Multisizer II (manufactured by Beckman Coulter, Inc.).

It is preferable that the toner particles have a pseudo-spherical shape from the viewpoints of improving developability and transfer efficiency and high image quality. The sphericity of the toner particles is represented by the shape factor SF1 of the following expression. The average of the

shape factors SF1 (average shape factor) of the toner particles used in the exemplary embodiment is preferably less than 145, more preferably equal to or greater than 115 and less than 140, and still more preferably equal to or greater than 120 and less than 140. When the average of the shape factors SF1 is less than 145, excellent transfer efficiency is obtained and image quality is high.

$$SF1 = \frac{(ML)^2}{A} \times \frac{\pi}{4} \times 100 \quad \text{Expression 1}$$

In the above expression, ML represents the maximum lengths of the respective toner particles and A represents the projection areas of the respective toner particles.

The average of the shape factors SF1 (average shape factor) is obtained by inputting 1000 toner images magnified 250 times to an image analyzer (LUZEX III, manufactured by Nireco Corporation) through an optical microscope, calculating the SF1 values of the respective particles from the maximum lengths and projection areas thereof, and obtaining the average thereof.

## Electrostatic Charge Image Developer

The electrostatic charge image developing toner according to the exemplary embodiment is preferably used as an electrostatic charge image developer.

The electrostatic charge image developer according to the exemplary embodiment is not particularly limited as long as it contains the electrostatic charge image developing toner according to the exemplary embodiment, and the configuration of components thereof is appropriately changed according to the purpose. A single-component electrostatic charge image developer in which the electrostatic charge image developing toner according to the exemplary embodiment is used alone or a two-component electrostatic charge image developer in which the electrostatic charge image developing toner according to the exemplary embodiment is used in combination with a carrier is prepared.

In the single-component developer, a method is used in which toner particles are charged by performing triboelectric charging using a development sleeve or a charging member and a toner image is developed according to an electrostatic latent image.

In the exemplary embodiment, a development method is not particularly specified, but two-component development is preferable. In addition, a carrier is not particularly specified as long as the above-described conditions are satisfied. Examples of a core material of a carrier include magnetic metals such as iron, steel, nickel, or cobalt; an alloy of the above-described metal and manganese, chromium, rare-earth elements, or the like; and magnetic oxides such as ferrite or magnetite. However, from the viewpoints of surface nature and resistance of a core material, ferrite, in particular, an alloy with manganese, lithium, strontium, magnesium, or the like is preferable.

It is preferable that the surface of the core material of the carrier used in the exemplary embodiment be coated with resin. The resin is not particularly limited and is appropriately selected according to the purpose. Examples of the resin include well-known resin such as polyolefin resin such as polyethylene or polypropylene; polyvinyl resin and polyvinylidene resin such as polystyrene, acrylic resin, polyacrylonitrile, polyvinyl acetate, polyvinyl alcohol, polyvinyl butyral, polyvinyl chloride, polyvinyl carbazole, polyvinyl ether, or polyvinyl ketone; vinyl chloride-vinyl acetate copolymer; styrene-acrylic acid copolymer; straight silicone

resin having an organosiloxane bond or a modified product thereof; fluororesin such as polytetrafluoroethylene, polyvinyl fluoride, polyvinylidene fluoride, or polychlorotrifluoroethylene; silicone resin; polyester; polyurethane; polycarbonate; phenol resin; amino resin such as urea formaldehyde resin, melamine resin, benzoguanamine resin, urea resin, or polyamide resin; and epoxy resin. These examples may be used alone or in a combination of two or more kinds thereof. In the exemplary embodiment, it is preferable that, among the above resins, at least fluororesin and/or silicone resin be used. When at least fluororesin and/or silicone resin is used as the resin, an effect of suppressing carrier contamination (impaction) caused by toner or an external additive is high, which is preferable.

In a coating layer formed by the resin, it is preferable that resin particles and/or conductive particles be dispersed in the resin. Examples of the resin particles include thermoplastic resin particles and thermosetting resin particles. Among these, thermosetting resin particles are preferable from the viewpoint of increasing hardness relatively easily and resin particles of nitrogen-containing resin which contains a nitrogen atom are preferable from the viewpoint of imparting a negative charging property to toner. In addition, the resin particles may be used alone or in a combination of two or more kinds thereof. The average particle size of the resin particles is preferably from 0.1  $\mu\text{m}$  to 2  $\mu\text{m}$  and more preferably from 0.2  $\mu\text{m}$  to 1  $\mu\text{m}$ . When the average particle size of the resin particles is equal to or greater than 0.1  $\mu\text{m}$ , the dispersibility of the resin particles in the coating layer is excellent. In addition, when the average particle size of the resin particles is less than or equal to 2  $\mu\text{m}$ , it is difficult that the resin particles be desorbed from the coating layer.

Examples of the conductive particles include metal particles such as particles of gold, silver, or copper; carbon black particles; and particles of titanium oxide, zinc oxide, barium sulfate, aluminum borate, potassium titanate or the like of which the surfaces are coated with tin oxide, carbon black, metal, or the like. The conductive particles are used alone or in a combination of two or more kinds thereof. Among these, carbon black particles are preferable from high preparation stability, low cost, and high conductivity. The kind of carbon black is not particularly limited, but carbon black having a DSP oil absorption of 50 ml/100 g to 250 ml/100 g is preferable due to its excellent preparation stability. The amount of the resin, the resin particles, and the conductive particles which coat the surface of the core material is preferably from 0.5% by weight to 5.0% by weight and more preferably from 0.7% by weight to 3.0% by weight.

A method of forming the coating layer is not particularly limited. For example, there is a method which uses a coating layer-forming solution which contains the resin particles such as cross-linked resin particles and/or the conductive particles; and the resin such as styrene acrylic resin, fluororesin, silicone resin or the like as a matrix resin in a solvent.

Specific examples thereof include a dipping method in which the core material of the carrier is dipped in the coating layer-forming solution, a spray method in which the coating layer-forming solution is sprayed on the surface of the core material of the carrier, and a kneader coater method in which the core material of the carrier and the coating layer-forming solution are mixed in a state where the core material is floated by flowing air and a solvent is removed. Among these, in the exemplary embodiment, the kneader coater method is preferable.

The solvent used for the coating layer-forming solution is not particularly limited as long as only the resin as a matrix resin may be dissolved therein. The solvent is selected from

well-known solvents, and examples thereof include aromatic hydrocarbons such as toluene or xylene; ketones such as acetone or methyl ethyl ketone; and ethers such as tetrahydrofuran or dioxane. When the resin particles are dispersed in the coating layer, the resin particles and the resin as a matrix resin are uniformly dispersed in a thickness direction thereof and in a circumference direction of the carrier surface. Accordingly, even if the carrier is used over a long period of time and the coating layer is abraded, the same surface as that before use is maintained all the time and an excellent charge-imparting property for the toner is maintained over a long period of time. When the conductive particles are dispersed in the coating layer, the conductive particles and the resin as a matrix resin are uniformly dispersed in a thickness direction thereof and in a tangent direction of the carrier surface. Accordingly, even if the carrier is used over a long period of time and the coating layer is abraded, the same surface as that before use is maintained all the time and deterioration of the carrier is prevented over a long period of time. In addition, when the resin particles and the conductive particles are dispersed in the coating layer, the same effects as above are exhibited at the same time.

The electrical resistance of the entire magnetic carrier formed as above in a magnetic brush state under an electric field of  $10^4$  V/cm is preferably from  $10^8$   $\Omega\text{cm}$  to  $10^{13}$   $\Omega\text{cm}$ . When the electrical resistance of the magnetic carrier is equal to or greater than  $10^8$   $\Omega\text{cm}$ , the attachment of the carrier to an image portion on an image holding member is suppressed and a brush mark is barely formed. When the electrical resistance of the magnetic carrier is less than or equal to  $10^{13}$   $\Omega\text{cm}$ , an edge effect is suppressed and thus a high-quality image may be obtained.

In this case, the electrical resistance (volume resistivity) is measured as follows.

On a lower polar plate of measurement equipment which is a pair of circular polar plates having a size of  $20\text{ cm}^2$  (made of steel) which is connected to an electrometer (trade name: KEITHLEY 610C, manufactured by Keithley Instruments Inc.) and a high voltage power supply (trade name: FLUKE 415B, manufactured by Fluke Corporation), samples are placed to form an approximately 1 mm to 3 mm-thick flat layer. Next, an upper polar plate is placed on the samples and a 4 kg weight is placed on the upper polar plate in order to eliminate the gap between the samples. In this state, the thickness of the sample layer is measured. Next, an electric current value is measured by applying voltage to both of the polar plates and the volume resistivity is calculated according to the following expression.

$$\text{Volume Resistivity} = \frac{\text{Applied Voltage} \times 20}{(\text{Current Value} - \text{Initial Current Value}) \times \text{Sample Thickness}}$$

In the expression above, Initial Current Value represents a current value when the applied voltage is 0 and Current Value represents a measured current value.

With regard to the mixing ratio of the toner and the carrier according to the exemplary embodiment in the two-component electrostatic charge image developer, the amount of the toner is 2 parts by weight to 10 parts by weight with respect to the 100 parts by weight of the carrier. In addition, the preparation method of the developer is not particularly limited, and, for example, a method of mixing the components using a V-blender or the like is used.

#### Image Forming Method

In addition, the electrostatic charge image developer (electrostatic charge image developing toner) is used for an image forming method for electrostatic charge image development (electrophotography).

The image forming method according to the exemplary embodiment includes a charging process of charging a surface of an image holding member; a latent image forming process of forming an electrostatic latent image on the surface of the image holding member; a developing process of forming a toner image by developing the electrostatic latent image, which is formed on the surface of the image holding member, using a developer; and a transfer process of transferring the formed toner image onto a recording medium, and may further include a fixing process of fixing the toner image transferred onto the surface of recording medium; and a cleaning process of cleaning an electrostatic charge image developer which remains on the image holding member. In this method, as the developer, the electrostatic charge image developing toner according to the exemplary embodiment or the electrostatic charge image developer according to the exemplary embodiment may be used.

The respective processes are well-known general processes and disclosed in, for example, JP-A-56-40868 and JP-A-49-91231. The image forming method according to the exemplary embodiment may be performed using well-known image forming apparatuses such as copying machines or fax machines.

In the latent image forming process, an electrostatic latent image is formed on the image holding member (photoreceptor).

In the developing process, the electrostatic latent image is developed by a developer layer on a developer holding member and thus a toner image is formed. The developer layer is not particularly limited as long as it contains the electrostatic charge image developing toner according to the exemplary embodiment.

In the transfer process, the toner image is transferred onto a transfer medium. In addition, as the transfer medium in the transfer process, for example, an intermediate transfer medium and a recording medium such as paper are used.

In the fixing process, for example, there is used a method of fixing a toner image, which is transferred onto transfer paper, using a heating roller fixing device in which the temperature of a heating roller is set to be constant, and forming a duplicate image.

In the cleaning process, an electrostatic charge image developer remaining on the image holding member is cleaned.

In addition, in the cleaning process of the image forming method according to the exemplary embodiment, it is preferable that an electrostatic charge image developer remaining on the image holding member be removed by a cleaning blade.

As the recording medium, well-known recording media such as paper or OHP sheets which are used for electrophotographic copying machines or printers are used, and preferable examples thereof include coated paper in which the surface of plain paper is coated with resin or the like and art paper for printing.

The image forming method according to the exemplary embodiment may further include a recycling process. In the recycling process, the electrostatic charge image developing toner, which is recovered in the cleaning process, is transferred to the developer layer. The image forming method including the recycling process is performed using an image forming apparatus such as toner recycling system type copying machines or fax machines. In addition, a recycling system in which development and toner recovery are performed at the same time may be adopted.

#### Image Forming Apparatus

The image forming apparatus according to the exemplary embodiment includes an image holding member; a charging unit that charges a surface of the image holding member; a latent image forming unit that forms an electrostatic latent image on the surface of the image holding member; a developing unit that forms a toner image by developing the electrostatic latent image, which is formed on the surface of the image holding member, using a developer; and a transfer unit that transfers the formed toner image onto a recording medium, and may further include a fixing unit that fixes the toner image transferred onto the surface of the recording medium; and a cleaning unit that cleans the image holding member. In this apparatus, as the developer, the electrostatic charge image developing toner according to the exemplary embodiment or the electrostatic charge image developer according to the exemplary embodiment may be used.

The image forming apparatus according to the exemplary embodiment is not particularly limited as long as it includes at least the image holding member, the charging unit, the exposure unit, the developing unit, the transfer unit, and the cleaning unit, but optionally, may further include the fixing unit or an erasing unit.

The transfer unit may perform transfer twice or more using an intermediate transfer medium. In addition, as the transfer medium of the transfer unit, for example, an intermediate transfer medium and a recording medium such as paper are used.

For the image holding member and the respective units, the components described for the respective processes of the image forming method may be preferably used. As the respective units, well-known units of image forming apparatuses may be used. In addition, the image forming apparatus according to the exemplary embodiment may include other units or devices except the above-described components. In addition, the image forming apparatus according to the exemplary embodiment may operate plural units of the above-described units at the same time.

In addition, as the cleaning unit that cleans an electrostatic charge image developer remaining on the image holding member, for example, a cleaning blade, a cleaning brush, and the like are used, but a cleaning blade is preferable.

Preferable examples of material of the cleaning blade include urethane rubber, neoprene rubber, and silicone rubber.

#### Toner Cartridge, Developer Cartridge, and Process Cartridge

A toner cartridge according to the exemplary embodiment includes a toner containing chamber that accommodates at least the electrostatic charge image developing toner according to the exemplary embodiment.

A developer cartridge according to the exemplary embodiment includes a developer containing chamber that accommodates at least the electrostatic charge image developer according to the exemplary embodiment.

In addition, a process cartridge according to the exemplary embodiment accommodates an electrostatic charge image developer and includes a developer holding member that holds and carries the electrostatic charge image developer. It is preferable that the process cartridge according to the exemplary embodiment include the developing unit that forms a toner image by developing an electrostatic latent image, which is formed on the surface of the image holding member, using the electrostatic charge image developing toner or the electrostatic charge image developer and at least one selected from a group consisting of the image holding member, the charging unit that charges the surface of the image holding member; and the cleaning unit that removes toner remaining

on the surface of the image holding member, in which at least the electrostatic charge image developing toner according to the exemplary embodiment or the electrostatic charge image developer according to the exemplary embodiment is accommodated.

It is preferable that the toner cartridge according to the exemplary embodiment be detachable from an image forming apparatus. That is, in the image forming apparatus from which the toner cartridge is detachable, the toner cartridge according to the exemplary embodiment accommodating the toner according to the exemplary embodiment is preferably used.

The developer cartridge according to the exemplary embodiment is not particularly limited as long as it contains an electrostatic charge image developer containing the electrostatic charge image developing toner according to the exemplary embodiment. For example, the developer cartridge is detachable from an image forming apparatus including the developing unit and accommodates, as a developer which is supplied to this developing unit, the electrostatic charge image developer containing the electrostatic charge image developing toner according to the exemplary embodiment.

In addition, the developer cartridge may accommodate a toner and a carrier. Alternatively, a cartridge accommodating a toner alone and a cartridge accommodating a carrier alone may be provided separately.

It is preferable that the process cartridge according to the exemplary embodiment be detachable from an image forming apparatus.

In addition, optionally, the process cartridge according to the exemplary embodiment may further include other units such as an erasing unit.

As the toner cartridge and the process cartridge, well-known configurations may be adopted, for example, configurations disclosed in JP-A-2008-209489 and JP-A-2008-233736 may be referred to.

## EXAMPLES

Hereinafter, the exemplary embodiment will be described in detail with reference to Examples, but is not limited to Examples. In the following description, "part" represents "part by weight" unless specified otherwise.

### Measurement of Mw and Mn of Resin

The weight average molecular weight (Mw) and the number average molecular weight (Mn) of a resin are measured and calculated using GPC (Gel Permeation Chromatography). Specifically, HLC-8120 (manufactured by TOSOH CORPORATION) is used for GPC, TSK gel Super HM-M (manufactured by TOSOH CORPORATION, 15 cm) is used as a column, and resin is dissolved in an organic solvent such as tetrahydrofuran (THF) for measurement. Next, the molecular weight of the resin is calculated using a molecular weight calibration curve prepared from monodisperse polystyrene standard samples.

### Volume Average Particle Size of Resin Particles, Colorant Particles and the Like

The volume average particle size of the resin particles, the colorant particles, and the like are measured using a laser diffraction particle size analyzer (manufactured by HORIBA, Ltd., LA-700).

### Measurement Method of Melting Temperature and Glass Transition Temperature of Resin

The melting temperature of crystalline polyester resin and the glass transition temperature (Tg) of amorphous polyester resin are obtained by a main maximum endothermic peak

which is measured using a differential scanning calorimeter (DSC-7, manufactured by PerkinElmer Inc.) in accordance with ASTM D3418-8. The temperature correction of a detection portion in this device (DSC-7) is performed using the melting temperatures of indium and zinc and the quantity of heat is corrected using the heat of fusion of indium. The samples are put in an aluminum pan, an empty pan is set for reference, followed by heating at a temperature rise rate of 10° C./min and measurement is performed.

### 10 Measurement Method of Volume Average Particle Size of Toner Particles

The volume average particle size of the toner particles is measured using a Coulter Multisizer II (manufactured by Beckman Coulter, Inc.). ISOTON-II (manufactured by Beckman Coulter, Inc.) is used as an electrolytic solution.

As the measurement method, first, a surfactant is used as a dispersant, and preferably, 0.5 mg to 50 mg of measurement samples are added to 2 ml of 5% aqueous sodium alkylbenzene sulfonate solution. This solution is added to 100 ml to 20 150 ml of the electrolytic solutions. The electrolytic solutions in which the measurement samples are suspended are dispersed using an ultrasonic disperser for approximately 1 minute, the particle size distribution of 2.0 µm to 60 µm particles is measured using Coulter Multisizer II with an aperture having an aperture size of 100 µm. The number of particles measured is 50,000.

The cumulative distribution of the measured particle size distribution from a smaller particle size side in terms of weight and volume is drawn in a divided particle size range 30 (channel). A particle size, which is an accumulated value of 50% in the cumulative distribution, is defined as the weight average particle size and the volume average particle size. Measurement of Glass Transition Temperature of Resin Particles in Resin Dispersion or Resin

35 The glass transition temperature Tg of resin is measured using a differential scanning calorimeter (DSC-50, manufactured by Shimadzu Corporation).

### Preparation of Toner Particles

### Preparation of Respective Dispersions

### 40 Preparation of Crystalline Polyester Resin Particle Dispersion 1

260 parts of 1,12-dodecane dicarboxylate, 165 parts of 1,10-decanediol, and 0.035 part of tetrabutoxy titanate as a catalyst are put into a heated and dried three-necked flask, 45 followed by reduction in the inner pressure of a vessel and reflux at 180° C. for 6 hours in an inert gas atmosphere of nitrogen gas under mechanical stirring. Then, the temperature is slowly raised to 220° C. through reduced-pressure distillation, followed by stirring for 2 and 3 hours. When the resultant becomes viscous, reduced-pressure distillation is stopped and air cooling is performed. As a result, Crystalline polyester resin 1 is obtained.

55 The weight average molecular weight (Mw) of Crystalline polyester resin 1 obtained above is 12,000 when measured in the above-described method. In addition, the melting temperature of Crystalline polyester resin 1 obtained above is 72° C. when measured using differential scanning calorimetry (DSC) in the above-described measurement method.

Next, 180 parts of Crystalline polyester resin 1 and 580 parts of deionized water are put into a stainless steel beaker and heated to 95° C. in a hot bath. When Crystalline polyester resin 1 is melted, stirring is performed at 8,000 rpm using a homogenizer (manufactured by IKA Japan K. K., ULTRA-TURRAX T50) and, at the same time, dilute ammonia water 60 is added thereto to adjust the pH value to 7.0. Next, 20 parts of aqueous solution in which 0.8 part of anionic surfactant (manufactured by DAI-ICHI KOGYO SEIYAKU CO., LTD.,

NEOGEN R) is diluted is added dropwise, followed by emulsification and dispersion. As a result, Crystalline polyester resin particle dispersion 1 with a volume average particle size of 0.24  $\mu\text{m}$  (concentration of resin particles: 12.5% by weight) is prepared.

Preparation of Amorphous Polyester Resin Particle Dispersion 1

73 parts of dimethyl adipate, 182 parts of dimethyl terephthalate, 217 parts of ethylene oxide adduct of bisphenol A, 41 parts of ethylene glycol, and 0.038 part of tetrabutoxy titanate as a catalyst are put into a heated and dried two-necked flask. Nitrogen gas is put into a vessel to maintain an inert gas atmosphere, followed by heating under stirring and a copolycondensation reaction at 160° C. for about 7 hours. Then, the resultant is heated to 220° C. and held for 3.5 hours while slowly reducing the pressure to 10 Torr. The pressure is temporarily returned to normal pressure, 9 parts of trimellitic anhydride is added, the pressure is slowly reduced to 10 Torr again, and the resultant is held for 1 hour. As a result, Amorphous polyester resin 1 is synthesized.

The glass transition temperature of Amorphous polyester resin 1 thus obtained is 58° C. when measured using differential scanning calorimeter (DSC) in the above-described measurement method. The weight average molecular weight (Mw) of Amorphous polyester resin 1 obtained above is 11,000 when measured using GPO in the above-described method.

Next, 115 parts of Amorphous polyester resin 1 and 180 parts of deionized water, and 5 parts of anionic surfactant (manufactured by DAI-ICHI KOGYO SEIYAKU CO., LTD., NEOGEN R) are mixed and heated to 120° C., sufficiently dispersed using a homogenizer (manufactured by IKA Japan K.K, ULTRA-TURRAX T50), followed by dispersion using a pressure discharge type Gaulin homogenizer by for 1 hours. As a result, Amorphous polyester resin particle dispersion 1 (concentration of resin particles: 40% by weight) is prepared.

Preparation of Styrene-Acrylic Resin Dispersion 1

Oil Layer 1

Styrene (manufactured by Wako Pure Chemical Industries): 32 parts

n-butyl acrylate (manufactured by Wako Pure Chemical Industries): 8 parts

$\beta$ -carboxyethyl acrylate (manufactured by Rhodia Nicca Ltd.): 1.2 parts

Dodecanthiol (manufactured by Wako Pure Chemical Industries): 0.5 part

Water Layer 1

Ion exchange water: 17.0 parts

Anionic surfactant (sodium alkylbenzenesulfonate, manufactured by Rhodia): 0.50 part

Water Layer 2

Ion exchange water: 40 parts

Anionic surfactant (sodium alkylbenzenesulfonate, manufactured by Rhodia): 0.06 part

Ammonium persulfate (manufactured by Wako Pure Chemical Industries): 0.4 part

The above components of Oil layer and Water layer 1 are put into a flask, stirred, and mixed to obtain a monomer-emulsified dispersion. The above components of Water layer 2 are put into a reaction vessel. The inside of the vessel is sufficiently substituted with nitrogen and heated in an oil bath under stirring until the temperature in the reaction system reaches 75° C.

The monomer-emulsified dispersion is slowly added dropwise into the reaction vessel over 3 hours for emulsion polymerization. After the dropwise addition, polymerization is

continued at 75° C. and stopped after 3 hours. As a result, Styrene-acrylic resin dispersion 1 is obtained.

In Styrene-acrylic resin dispersion 1 thus obtained, the volume average particle size of resin particles is 330 nm and the weight average molecular weight (Mw) is 12,500 when measured using the above-described method. In addition, the galls transition temperature is 52° C. when measured using differential scanning calorimeter (DSC) in the above-described measurement method.

10 Preparation of Colorant Dispersion

100 parts of cyan pigment (manufactured by Dainichiseika&Chemicals Mfg. Co., Ltd., C.I. Pigment Blue 15:3, copper phthalocyanine), 15 parts of anionic surfactant (manufactured by DAI-ICHI KOGYO SEIYAKU CO., LTD., 15 NEOGEN R), and 300 parts of ion exchange water are mixed, dispersed for 10 minutes using a homogenizer (manufactured by TKA Japan K.K, ULTRA-TURRAX T50), and put into a circulation-type supersonic dispersing machine (manufactured by NISSEI Corporation, RUS-600 TCVP). As a result, 20 Colorant dispersion is obtained.

In Colorant dispersion thus obtained, the volume average particle size of the colorant (cyan pigment) is 0.17  $\mu\text{m}$  when measured using a laser diffraction particle size analyzer in the above-described measurement method. In addition, the solid content of the cyan colorant dispersion is 24% by weight.

Preparation of Release agent Dispersion

95 parts of Fischer-Tropsch wax FNP92 (melting temperature: 92° C., manufactured by NIPPON SERIO CO., LTD.), 3.6 parts of anionic surfactant (manufactured by DAI-ICHI 30 KOGYO SEIYAKU CO., LTD., NEOGEN R), 360 parts of ion exchange water are mixed and heated to 100° C., sufficiently dispersed using a homogenizer (manufactured by IKA Japan K.K, ULTRA-TURRAX T50), followed by dispersion using a pressure discharge type Gaulin homogenizer. As a 35 result, Release agent dispersion is obtained.

In Release agent dispersion thus obtained, the volume average particle size of the release agent is 0.24  $\mu\text{m}$  when measured using a laser diffraction particle size analyzer in the above-described measurement method. In addition, the solid content of Release dispersion is 20% by weight.

Preparation of Toner Particles 1

104.4 parts of Crystalline polyester resin particle dispersion 1, 336.1 parts of Amorphous polyester resin particle dispersion 1, 45.4 parts of Colorant dispersion, 115.3 parts of 45 Release agent dispersion, and 484 parts of deionized water are put into a stainless steel round flask, and sufficiently mixed and dispersed using ULTRA-TURRAX T50. Next, 0.37 part of polyaluminium chloride is added thereto and dispersion is continued using ULTRA-TURRAX T50. Furthermore, the flask is heated to 52° C. in a heating oil bath under stirring. After this state is held for 3 hours at 52° C., 175 parts of Amorphous polyester resin particle dispersion 1 is slowly added thereto. Next, the pH value of the system is 50 adjusted to 8.5 using 0.5 N aqueous sodium hydroxide solution. Then, the stainless steel flask is sealed, heated to 90° C. while being stirred using a magnetic seal, and held for 3 hours. After a reaction is stopped, the resultant is cooled, filtrated, sufficiently washed with ion exchange water, followed by solid-liquid separation with a Nutsche vacuum filter. The resultant is dispersed again in 3,000 parts of ion 55 exchange water at 30° C., stirred for 15 minutes at 300 rpm, and washed. The above process is repeated five more times. When the pH value of the filtrate is 6.85, the electrical conductance is 8.2  $\mu\text{S}/\text{cm}$ , and the surface tension is 70.5 N/m,

60 washing is stopped, followed by solid-liquid separation with a Nutsche vacuum filter using No. 5A filter paper and vacuum drying for 12 hours. As a result, Toner particles 1 are obtained.

## 25

The glass transition temperature of Toner Particles 1 thus obtained is 54.0° C. when measured in the above-described method. The volume average particle size of Toner Particles 1 is 5.8  $\mu\text{m}$  when measured in the above-described measurement method. In addition, the average circularity of Toner Particles 1 is 0.959 when measured in the method.

Average circularity is obtained by measuring the sphericities of 5,000 particles using a flow particle image analyzer FPIA-3000 (manufactured by SYSMEX CORPORATION) and obtaining the number-average value thereof.

The above average circularity is obtained by analyzing images of toner particles in predetermined numbers, calculating the circularity of the respective imaged toner particles according to the expression below, and obtaining the average value thereof.

$$\text{Circularity} = \frac{\text{Perimeter of Circle with Equivalent Diameter}}{\text{Perimeter}} = \frac{2 \times (A \times \pi)^{1/2}}{P}$$

In the above expression, A represents a projection area and PM represents a perimeter.

## Preparation of Toner Particles 2

Styrene-Acrylic Resin Dispersion 1: 70 parts

Colorant dispersion: 14 parts

Release agent dispersion: 22 parts

Polyaluminium chloride: 0.14 part

The above components are put into a stainless steel round flask, and sufficiently mixed and dispersed using ULTRA-TURRAX T50. Next, 0.32 part of polyaluminium chloride is added thereto and dispersion is continued using ULTRA-TURRAX T50. Furthermore, the flask is heated to 47° C. in a heating oil bath under stirring. After this state is held for 60 minutes at 47° C., 30 parts of Styrene-Acrylic Resin Dispersion 1 is slowly added thereto.

Next, the pH value of the system is adjusted to 6.0 using 0.5 mol/L of aqueous sodium hydroxide solution. Then, the stainless steel flask is sealed, heated to 96° C. while being stirred using a magnetic seal, and held for 3.5 hours. After a reaction is stopped, the resultant is cooled, filtrated, sufficiently washed with ion exchange water, followed by solid-liquid separation with a Nutsche vacuum filter. The resultant is dispersed again in 3000 parts of ion exchange water at 40° C., stirred for 15 minutes at 300 rpm, and washed.

The above process is repeated five more times. When the pH value of the filtrate is 7.01, the electrical conductance is 9.7  $\mu\text{S}/\text{cm}$ , and the surface tension is 71.2 N/m, washing is stopped, followed by solid-liquid separation with a Nutsche vacuum filter using No. 5A filter paper and vacuum drying for 12 hours. As a result, Toner particles 2 are obtained.

The volume average particle size of Toner Particles 2 thus obtained is 5.7  $\mu\text{m}$  when measured in the above-described method. In addition, the average circularity of Toner Particles 2 is 0.957 when measured in the above-described method.

## Preparation of Toner Particles 3

A mixture of 100 parts of styrene-butyl acrylate copolymer (weight average molecular weight  $M_w=150,000$ , copolymerization ratio=80:20), 5 parts of carbon black (Mogul L, manufactured by Cabot Corporation), and 6 parts of carnauba wax is kneaded using an extruder and finely pulverized using a jet mill, followed by spheronization with warm air using Kryptron (manufactured by Kawasaki Heavy Industries, Ltd.) and classification using a wind classifier. As a result, Toner particles 3 having an average particle size of 6.2  $\mu\text{m}$  are obtained.

## Preparation of Treatment External Additive 1

10 parts of hydrophobic fumed silica R8200 (average particle size: 12 nm, manufactured by Nippon Aerosil Co., Ltd.) and 2.5 parts of 1,1,3,5,5-pentaphenyl-1,3,5-trimethyl pentanetrisiloxane are mixed using a sample mill. As a result, Treatment external additive 1 is obtained.

## 26

tanetrisiloxane are mixed using a sample mill. As a result, Treatment external additive 1 is obtained.

## Preparation of Treatment External Additive 2

10 parts of hydrophobic fumed silica R8200 (average particle size: 12 nm, manufactured by Nippon Aerosil Co., Ltd.) and 2.5 parts of 1,1,5,5-tetraphenyl-1,3,3,5-tetramethyl pentanetrisiloxane are mixed using a sample mill. As a result, Treatment external additive 2 is obtained.

## Preparation of Treatment External Additive 3

10 parts of hydrophobic fumed silica R8200 (average particle size: 12 nm, manufactured by Nippon Aerosil Co., Ltd.) and 1.0 part of 1,1,3,5,5-pentaphenyl-1,3,5-trimethyl pentanetrisiloxane are mixed using a sample mill. As a result, Treatment external additive 3 is obtained.

## Preparation of Treatment External Additive 4

10 parts of hydrophobic titanium oxide JMT-150AO (average particle size: 15 nm, manufactured by Tayca Corporation) and 2.5 part of 1,1,3,5,5-pentaphenyl-1,3,5-trimethyl pentanetrisiloxane are mixed using a sample mill. As a result, Treatment external additive 4 is obtained.

## Preparation of Treatment External Additive 5

10 parts of hydrophobic fumed silica R8200 (average particle size: 12 nm, manufactured by Nippon Aerosil Co., Ltd.) and 10.0 parts of 1,1,3,5,5-pentaphenyl-1,3,5-trimethyl pentanetrisiloxane are mixed using a sample mill. As a result, Treatment external additive 5 is obtained.

## Preparation of Treatment External Additive 6

10 parts of hydrophobic fumed silica R8200 (average particle size: 12 nm, manufactured by Nippon Aerosil Co., Ltd.) and 2.5 parts of octamethyl trisiloxane are mixed using a sample mill. As a result, Treatment external additive 6 is obtained.

## Preparation of Treatment External Additive 7

10 parts of hydrophobic fumed silica R8200 (average particle size: 12 nm, manufactured by Nippon Aerosil Co., Ltd.) and 2.5 parts of 1,1,1,3,3,5,5-heptamethyl-5-phenyl pentanetrisiloxane are mixed using a sample mill. As a result, Treatment external additive 7 is obtained.

## Preparation of Treatment External Additive 8

10 parts of hydrophobic fumed silica R8200 (average particle size: 12 nm, manufactured by Nippon Aerosil Co., Ltd.) and 2.5 parts of dimethyl silicone oil KF-96-50cs (manufactured by Shin-Etsu Chemical Co., Ltd.) are mixed using a sample mill. As a result, Treatment external additive 8 is obtained.

## Example 1

## Preparation of External Additive-Added Toner 1

2 parts of Treatment external additive 1 are added with respect to 100 parts of Toner particles 1 and blended using a sample mill. As a result, External additive-added toner 1 is obtained.

## Preparation of Developer 1

External additive-added toner 1 is weighed and added to ferrite carrier particles having a volume average particle size of 50  $\mu\text{m}$  which is coated with 1% by weight of polymethyl methacrylate (manufactured by Soken Chemical&Engineering Co., Ltd.) such that the toner concentration is 5% by weight, followed by stirring with a V-blender for 30 minutes and mixing. As a result, Developer 1 is prepared.

Using Developer 1 thus obtained, the following image printing test and cleaning property test are conducted. The results thereof are shown in Table 1.

27

Image Printing Test (Examination of Background Fogging Due to Electric Charge Leakage)

In a high-humidity environment of 30° and 88%, a test is conducted over two days, in which 30,000 images of The Imaging Society of Japan Test Chart No. 8 (5%) are printed on A4-sized plain paper (manufactured by Fuji Xerox Co., Ltd., C2 paper) using a modified DocuCenterColor 400 machine (manufactured by Fuji Xerox Co., Ltd.). On Day one, 20,000 images are continuously printed and an image of The Imaging Society of Japan Test Chart No. 1 is printed in the first operation in the morning of the following day. Then, 10,000 images are further continuously printed over one day. After 30,000 images in total are printed, an image of The Imaging Society of Japan Test Chart No. 1 is printed in the first operation in the morning of the following day for evaluation. In the evaluation, A to C are in an acceptable range.

A: Fogging is not found on an image and there is no problem with image quality. No toner scatter is found in the actual machine

B: Fogging is not found on an image but a small toner scatter is found in the actual machine

C: A small amount of fogging is found on an image and a toner scatter is found in the actual machine

D: Fogging and deterioration in the reproduction of a thin line are found on an image and a toner scatter is found in the actual machine

Cleaning Property (Examination of Cleaning Property for Toner Filming)

In a low-humidity environment of 20° and 15%, a test is conducted, in which 30,000 images of The Imaging Society of Japan Test Chart No. 8 (5%) are printed on A4-sized plain paper (manufactured by Fuji Xerox Co., Ltd., C2 paper) using a modified DocuCenterColor 400 machine (manufactured by Fuji Xerox Co., Ltd.). A photoreceptor is detached whenever 10,000 images are printed, and the surface of the photoreceptor and the surface of a printed image are visually inspected. The evaluation is conducted as follows and A to C are in an acceptable range. In addition, when evaluation result is D, the test is stopped at that stage. When evaluation result is one of A to C after 20,000 images are printed, it is determined that the toner has an excellent cleaning property as the toner according to the exemplary embodiment.

A: Foreign substances attached to a photoreceptor and a toner contamination on an image are not found by visual inspection

B: Foreign substances attached to a photoreceptor are found but a toner contamination on an image is not found

C: Foreign substances attached to a photoreceptor are found but a small toner contamination on an image is found

D: a toner contamination is found on the entire surface of a photoreceptor

Example 2

Preparation of External Additive-Added Toner 2

2 parts of Treatment external additive 2 are added with respect to 100 parts of Toner particles 1 and blended using a sample mill. As a result, External additive-added toner 2 is obtained.

Preparation of Developer 2

Developer 2 is obtained in the same preparation method as that of Developer 1, except that External additive-added toner 2 is used instead of External additive-added toner 1.

Using Developer 2 thus obtained, the same test as that of Example 1 is conducted. The results thereof are shown in Table 1.

28

Example 3

Preparation of External Additive-Added Toner 3

5 2 parts of Treatment external additive 3 are added with respect to 100 parts of Toner particles 1 and blended using a sample mill. As a result, External additive-added toner 3 is obtained.

10 Preparation of Developer 3

Developer 3 is obtained in the same preparation method as that of Developer 1, except that External additive-added toner 3 is used instead of External additive-added toner 1.

15 Using Developer 3 thus obtained, the same test as that of Example 1 is conducted. The results thereof are shown in Table 1.

Example 4

Preparation of External Additive-Added Toner 4

20 2 parts of Treatment external additive 4 are added with respect to 100 parts of Toner particles 1 and blended using a sample mill. As a result, External additive-added toner 4 is obtained.

Preparation of Developer 4

Developer 4 is obtained in the same preparation method as that of Developer 1, except that External additive-added toner 4 is used instead of External additive-added toner 1.

30 Using Developer 4 thus obtained, the same test as that of Example 1 is conducted. The results thereof are shown in Table 1.

Example 5

Preparation of External Additive-Added Toner 5

35 4 parts of Treatment external additive 5 are added with respect to 100 parts of Toner particles 1 and blended using a sample mill. As a result, External additive-added toner 5 is obtained.

40 Preparation of Developer 5

Developer 5 is obtained in the same preparation method as that of Developer 1, except that External additive-added toner 5 is used instead of External additive-added toner 1.

45 Using Developer 5 thus obtained, the same test as that of Example 1 is conducted. The results thereof are shown in Table 1.

Example 6

Preparation of External Additive-Added Toner 6

50 2 parts of Treatment external additive 1 are added with respect to 100 parts of Toner particles 2 and blended using a sample mill. As a result, External additive-added toner 6 is obtained.

Preparation of Developer 6

Developer 6 is obtained in the same preparation method as that of Developer 1, except that External additive-added toner 6 is used instead of External additive-added toner 1.

Using Developer 6 thus obtained, the same test as that of Example 1 is conducted. The results thereof are shown in Table 1.

#### Example 7

##### Preparation of External Additive-Added Toner 7

2 parts of Treatment external additive 1 are added with respect to 100 parts of Toner particles 3 and blended using a sample mill. As a result, External additive-added toner 7 is obtained.

##### Preparation of Developer 7

Developer 7 is obtained in the same preparation method as that of Developer 1, except that External additive-added toner 7 is used instead of External additive-added toner 1.

Using Developer 7 thus obtained, the same test as that of Example 1 is conducted. The results thereof are shown in Table 1.

#### Comparative Example 1

##### Preparation of External Additive-Added Toner 8

2 parts of Treatment external additive 6 is added with respect to 100 parts of Toner particles 1 and blended using a sample mill. As a result, External additive-added toner 8 is obtained.

##### Preparation of Developer 8

Developer 8 is obtained in the same preparation method as that of Developer 1, except that External additive-added toner 8 is used instead of External additive-added toner 1.

Using Developer 8 thus obtained, the same test as that of Example 1 is conducted. The results thereof are shown in Table 1.

#### Comparative Example 2

##### Preparation of External Additive-Added Toner 9

2 parts of Treatment external additive 7 are added with respect to 100 parts of Toner particles 1 and blended using a sample mill. As a result, External additive-added toner 9 is obtained.

Preparation of Developer 9

Developer 9 is obtained in the same preparation method as that of Developer 1, except that External additive-added toner 9 is used instead of External additive-added toner 1.

Using Developer 9 thus obtained, the same test as that of Example 1 is conducted. The results thereof are shown in Table 1.

##### Preparation of Developer 9

Developer 9 is obtained in the same preparation method as that of Developer 1, except that External additive-added toner 9 is used instead of External additive-added toner 1.

Using Developer 9 thus obtained, the same test as that of Example 1 is conducted. The results thereof are shown in Table 1.

#### Comparative Example 3

##### Preparation of External Additive-Added Toner 10

2 parts of hydrophobic fumed silica R8200 (average particle size: 12 nm, manufactured by Nippon Aerosil Co., Ltd.) are added with respect to 100 parts of Toner particles 1 and blended using a sample mill. As a result, External additive-added toner 10 is obtained.

##### Preparation of Developer 10

Developer 10 is obtained in the same preparation method as that of Developer 1, except that External additive-added toner 10 is used instead of External additive-added toner 1.

Using Developer 10 thus obtained, the same test as that of Example 1 is conducted. The results thereof are shown in Table 1.

#### Comparative Example 4

##### Preparation of External Additive-Added Toner 11

2 parts of Treatment external additive 8 are added with respect to 100 parts of Toner particles 1 and blended using a sample mill. As a result, External additive-added toner 11 is obtained.

##### Preparation of Developer 11

Developer 11 is obtained in the same preparation method as that of Developer 1, except that External additive-added toner 11 is used instead of External additive-added toner 1.

Using Developer 11 thus obtained, the same test as that of Example 1 is conducted. The results thereof are shown in Table 1.

TABLE 1

|           | Toner<br>Particles | Treatment<br>External<br>Additive | Siloxane Compound                                                 | Number of<br>Phenyl Groups<br>Represented<br>by R <sup>2</sup> to R <sup>7</sup> | Content of<br>Compound<br>Represented<br>by Formula (1)<br>in Toner | Evaluation<br>of Cleaning<br>Property for<br>Toner<br>Filming | Evaluation<br>of Background<br>Fogging due to<br>Electric<br>charge leakage |
|-----------|--------------------|-----------------------------------|-------------------------------------------------------------------|----------------------------------------------------------------------------------|---------------------------------------------------------------------|---------------------------------------------------------------|-----------------------------------------------------------------------------|
| Example 1 | Toner 1            | 1<br>Silica                       | 1,1,3,5,5-pentaphenyl-<br>1,3,5-trimethyl<br>pentanetrisiloxane   | 5                                                                                | 0.50 wt %                                                           | A                                                             | A                                                                           |
| Example 2 | Toner 1            | 2<br>Silica                       | 1,1,5,5-tetraphenyl-1,<br>3,3,5-tetramethyl<br>pentanetrisiloxane | 4                                                                                | 0.50 wt %                                                           | A                                                             | B                                                                           |
| Example 3 | Toner 1            | 3<br>Silica                       | 1,1,3,5,5-pentaphenyl-<br>1,3,5-trimethyl<br>pentanetrisiloxane   | 5                                                                                | 0.20 wt %                                                           | B                                                             | B                                                                           |
| Example 4 | Toner 1            | 4<br>Titanium<br>Oxide            | 1,1,3,5,5-pentaphenyl-<br>1,3,5-trimethyl<br>pentanetrisiloxane   | 5                                                                                | 0.50 wt %                                                           | A                                                             | B                                                                           |
| Example 5 | Toner 1            | 5<br>Silica                       | 1,1,3,5,5-pentaphenyl-<br>1,3,5-trimethyl<br>pentanetrisiloxane   | 5                                                                                | 4.0 wt %                                                            | B                                                             | B                                                                           |
| Example 6 | Toner 2            | 1<br>Silica                       | 1,1,3,5,5-pentaphenyl-<br>1,3,5-trimethyl<br>pentanetrisiloxane   | 5                                                                                | 0.50 wt %                                                           | A                                                             | A                                                                           |

TABLE 1-continued

|                          | Toner<br>Particles | Treatment<br>External<br>Additive | Siloxane Compound                                        | Number of<br>Phenyl Groups<br>Represented<br>by R <sup>2</sup> to R <sup>7</sup> | Content of<br>Compound<br>Represented<br>by Formula (1)<br>in Toner | Evaluation<br>of Cleaning<br>Property for<br>Toner<br>Filming | Evaluation of<br>Background<br>Fogging due to<br>Electric<br>charge leakage |
|--------------------------|--------------------|-----------------------------------|----------------------------------------------------------|----------------------------------------------------------------------------------|---------------------------------------------------------------------|---------------------------------------------------------------|-----------------------------------------------------------------------------|
| Example 7                | Toner 3            | 1<br>Silica                       | 1,1,3,5,5-pentaphenyl-1,3,5-trimethyl pentanetrisiloxane | 5                                                                                | 0.50 wt %                                                           | A                                                             | A                                                                           |
| Comparative<br>Example 1 | Toner 1            | 6<br>Silica                       | octamethyl trisiloxane                                   | 0                                                                                | 0.50 wt %                                                           | C                                                             | D                                                                           |
| Comparative<br>Example 2 | Toner 1            | 7<br>Silica                       | 1,1,1,3,3,5,5-heptamethyl-5-phenyl pentanetrisiloxane    | 1                                                                                | 0.50 wt %                                                           | B                                                             | D                                                                           |
| Comparative<br>Example 3 | Toner 1            | Silica                            | None                                                     | —                                                                                | —                                                                   | D                                                             | D                                                                           |
| Comparative<br>Example 4 | Toner 1            | 8<br>Silica                       | (Dimethyl Silicone<br>Oil)                               | —                                                                                | (0.50 wt %)                                                         | D                                                             | D                                                                           |

In Table 1, 1,1,3,5,5-pentaphenyl-1,3,5-trimethyl pentanetrisiloxane is a compound represented by Formula (A) below, 1,1,5,5-tetraphenyl-1,3,3,5-tetramethyl pentanetrisiloxane is a compound represented by Formula (B) below, octamethyl trisiloxane is a compound represented by Formula (C) below, and 1,1,1,3,3,5,5-heptamethyl-5-phenyl pentanetrisiloxane is a compound represented by Formula (D) below.

or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.



The foregoing description of the exemplary embodiments of the present invention has been provided for the purposes of illustration and description. It is not intended to be exhaustive

What is claimed is:

1. An electrostatic charge image developing toner comprising:  
toner particles containing a colorant, a binder resin, and a release agent; and  
an external additive,  
wherein the external additive contains inorganic particles which include a compound represented by Formula (1) below on the surfaces thereof.

(B) 40



(1)

wherein in Formula (1), R<sup>1</sup> and R<sup>8</sup> each independently represents an alkyl group, R<sup>2</sup> to R<sup>7</sup> each independently represents an alkyl group or a substituted or unsubstituted phenyl group, and at least three groups of R<sup>2</sup> to R<sup>7</sup> each independently represents a substituted or unsubstituted phenyl group.

2. The electrostatic charge image developing toner according to claim 1,

wherein the alkyl groups represented by R<sup>1</sup> and R<sup>8</sup> have from 1 to 20 carbon atoms.

3. The electrostatic charge image developing toner according to claim 1,

wherein a content of the compound is in the range of 0.16% by weight to 5% by weight with respect to the total weight of the toner.

4. The electrostatic charge image developing toner according to claim 1,

wherein 50% by area or more of the surfaces of the inorganic particles are coated with the compound.

5. The electrostatic charge image developing toner according to claim 1,

## 33

wherein the compound is selected from a group consisting of 1,1,3,5,5-pentaphenyl-1,3,5-trialkyl trisiloxane, 1,1,5,5-tetraphenyl-1,3,3,5-tetraalkyl trisiloxane, 1,1,3,3,5,5-hexaphenyl-1,5-dialkyl trisiloxane, 1,1,3,3,5-pentaphenyl-1,5,5-trialkyl trisiloxane, 1,1,3,5-tetraphenyl-1,3,5,5-tetraalkyl trisiloxane, 1,3,3,5-tetraphenyl-1,1,5,5-tetraalkyl trisiloxane, 1,3,5-triphenyl-1,1,3,5,5-pentaalkyl trisiloxane, and 1,1,5-triphenyl-1,3,3,5,5-pentaalkyl trisiloxane.

6. The electrostatic charge image developing toner according to claim 1,

wherein a volume average primary particle size of the inorganic particles is in the range of 3 nm to 500 nm.

7. The electrostatic charge image developing toner according to claim 1,

wherein a volume average primary particle size of the inorganic particles is in the range of 20 nm to 200 nm.

8. The electrostatic charge image developing toner according to claim 1,

wherein a content of inorganic particles having the compound on the surfaces thereof is in the range of 0.3% by weight to 10% by weight with respect to the total weight of the toner.

9. The electrostatic charge image developing toner according to claim 1,

wherein the toner particles contain from 2% by weight to 30% by weight of crystalline polyester resin with respect to the total weight of the toner particles.

10. An electrostatic charge image developer comprising:

the toner according to claim 1; and

a carrier.

11. The electrostatic charge image developer according to claim 10,

wherein a content of the compound is in the range of 0.16% by weight to 5% by weight with respect to the total weight of the toner.

12. A toner cartridge comprising:

a toner containing chamber that accommodates the electrostatic charge image developing toner according to claim 1.

13. A developer cartridge comprising:

a developer containing chamber that accommodates the electrostatic charge image developer according to claim 10.

14. A process cartridge for an image forming apparatus comprising:

## 34

a developer holding member that holds and carries an electrostatic charge image developer, wherein the electrostatic charge image developer is the electrostatic charge image developer according to claim 10.

15. The process cartridge for an image forming apparatus according to claim 14,

wherein a content of the compound is in the range of 0.16% by weight to 5% by weight with respect to the total weight of the toner.

16. An image forming apparatus comprising:

an image holding member;

a charging unit that charges a surface of the image holding member;

a latent image forming unit that forms an electrostatic latent image on the surface of the image holding member;

a developing unit that forms a toner image by developing the electrostatic latent image, which is formed on the surface of the image holding member, using a developer; and

a transfer unit that transfers the formed toner image onto a recording medium,

wherein the developer is the electrostatic charge image developer according to claim 10.

17. The image forming apparatus according to claim 16, wherein a content of the compound is in the range of 0.16% by weight to 5% by weight with respect to the total weight of the toner.

18. An image forming method comprising:

charging a surface of an image holding member; forming an electrostatic latent image on the surface of the image holding member;

forming a toner image by developing the electrostatic latent image, which is formed on the surface of the image holding member, using a developer; and transferring the formed toner image onto a recording medium,

wherein the developer is the electrostatic charge image developer according to claim 10.

19. The image forming method according to claim 18, wherein a content of the compound is in the range of 0.16% by weight to 5% by weight with respect to the total weight of the toner.

\* \* \* \* \*